

Nov. 21, 1972

D. S. DUSTIN

3,703,362

PRESENSITIZED LIGHT-SENSITIVE LETTERPRESS PRINTING MAKEREADY

Filed Jan. 17, 1972



FIG. 1



FIG. 2



FIG. 3



FIG. 4



FIG. 5

1

**3,703,362**  
**PRESENSITIZED LIGHT-SENSITIVE LETTERPRESS**  
**PRINTING MAKEREADY**

Daniel S. Dustin, Minneapolis, Minn., assignor to Minnesota Mining and Manufacturing Company, St. Paul, Minn.

Filed Jan. 17, 1972, Ser. No. 218,238  
Int. Cl. G03c 5/00, 11/00

U.S. Cl. 96—38.2

8 Claims

## ABSTRACT OF THE DISCLOSURE

Novel presensitized light-sensitive makeready sheet material for letterpress printing is provided. This sheet material is comprised of a flexible backing overlaid in ascending order with a thermoexpansive layer, a light-sensitive diazo resin layer, and an outer layer of a pigmented, water-insoluble, solvent-softenable polymeric compound.

## FIELD OF THE INVENTION

This invention relates to the art of makeready for letterpress printing, especially as related to letterpress printing wherein photopolymer relief printing plates are utilized.

## BACKGROUND OF THE INVENTION

In letterpress printing, an impression cylinder is commonly used to press a sheet, usually paper, against the inked face of a printing plate. The ink on the face of image of the printing plate, i.e., on the surface of raised printing elements, is thereby printed upon the sheet.

For highest quality letterpress printing, certain preliminary steps are required in readying the printing apparatus for operation. Makeready is a part of this preliminary procedure and, as used herein, involves selectively adjusting the impression pressure under which areas of the face of the printing plate and the impression cylinder meet or coat during printing. This selective adjustment of impression pressure affords prints which have dense solids, uniform, clean line copy, and in picture areas, a full range of half tones, from deep shadow areas to clean highlights, such as are desirable in encyclopedias, art magazines, and the like.

This adjustment of impression pressure can be accomplished by varying the thickness of packing on selected areas of the impression cylinder, commonly termed "overlay" makeready. Alternatively, or in conjunction with overlay makeready, pressure corrective material can be inserted beneath the mounting block on which a printing plate rests, termed "underlay" makeready, and/or between the printing plate and the mounting block, termed "interlay" makeready.

In this manner, impression pressure in solid tone printing areas is increased with respect to that in middle tone printing areas, the highlight or nonprinting areas receive the least pressure.

Consistent with conventional terminology, solid tone printing areas have a high tonal density, i.e., a high percentage of ink is contained per unit of surface area. Middle tone printing areas have a correspondingly lower tonal density, i.e., a lower percentage of ink is contained per unit of surface area. Nonprinting or highlight areas would of necessity have the least tonal density.

A novel makeready sheet material was the subject of Gergen and Wartman, U.S. Pat. No. 2,825,282, granted Mar. 4, 1958. This patent utilizes the selective expansion of a thermoexpansive layer of sheet material which is resistant to compression when expanded. In general, this sheet material is inked or printed with the general like-

2

ness of a printing plate and exposed to high-intensity radiant energy. Because the inked image area is absorptive of this radiant energy, a selective differential sustained expansion occurs. Upon cooling, the expanded material becomes hard and resistant to the compression pressures expected during the printing operation. The expanded sheet material is then placed in registration with the printing plate such that the greatest expansion areas coact with the solid tone areas of the printing plate, i.e., the thickness relief of the expanded sheet corresponds to the tone of the printing plate.

Since the advent of this makeready sheet material, printing plates or forms utilizing photopolymerization have been introduced in the printing field. Such plates are exposed through photographic negatives of the desired printed matter and developed, such that the image is retained on the form and nonimage areas are removed, thus providing a suitable relief printing plate.

Use of the makeready sheet material of the Gergen and Wartman patent with photopolymer relief printing plates requires the inking of the imaged and developed printing plate, the transfer of the inked image to the makeready sheet material, followed by selective expansion in the inked areas. Registration of the makeready material must be by some mechanical means, such as a mark or slit on the impression cylinder, to provide the exacting registration needed for high quality printing. In addition, overlay makeready, wherein the selective adjustment of impression pressure occurs through variation in thickness of impression cylinder packing, would normally be required since the image inked on the makeready sheet would be reverse reading from that of the printing plate.

This invention utilizes the basic principles of the Gergen and Wartman makeready sheet material, i.e., selective differential expansion of a thermoexpansive layer in image areas, and improves upon it by providing makeready sheet material which is light-sensitive. This allows the makeready material to be formed utilizing the same photographic negative used to image the photopolymer relief printing plate, without forming the photopolymer plate, registering the plate on a printing press, inking the plate, and transferring the inked image to the mounted makeready sheet. Thus, the makeready sheet of this invention can be developed and expanded independent of the printing plate preparation. Since the photographic negative used in the process normally contains registry marks for registration of the completed photopolymer printing plate, these same registry marks can be utilized in the makeready sheet, thereby greatly reducing registration time. Thus, the invention provides a substantial decrease in press set-up time, an extremely desirable feature from an economic standpoint.

## SUMMARY OF THE INVENTION

In accordance with the invention, there is provided a presensitized light-sensitive makeready sheet material comprising a flexible backing or carrier web on which there is overlaid: a selectively thermoexpansive layer comprising an at least temporarily thermosoftenable resin and uniformly distributed therethrough a heat-sensitive puffing agent capable of expanding this layer at least two mils in thickness when heated activated; a light-sensitive diazo resin sensitizer layer which becomes insoluble and firmly bonded to the thermoexpansive layer beneath it in light exposed image areas, the unexposed areas remaining soluble; and an outer actinic light-transmittable layer comprising a water-insoluble, solvent-softenable polymeric compound which has a pigment absorptive of infrared or equivalent high intensity radiant energy dispersed uniformly therethrough. Upon image-wise exposure, the light exposed portions of this outer layer become firmly bonded to the underlying diazo

resin layer and impervious to the action of a developing solution, while the unexposed areas are readily removable with the underlying unexposed sensitizer layer.

This makeready sheet material can be exposed to the same photographic negative used to expose the photopolymer relief printing plate, developed to reveal a pigmented image area absorptive of high-intensity radiant energy, and then expanded according to the methods taught by the Gergen and Wartman patent. This affords a makeready sheet material which can be processed independent of the photopolymer printing plate and does not have to be press mounted, as for ordinary proofing, etc., until final registration with the photopolymer printing plate, yet will provide the proper differential of impression pressure to yield high quality letterpress printing. Areas of the image-developed makeready sheet material containing a high tonal density or high percentage of pigment per unit surface area, i.e., solid or shadow tone areas, absorb a greater amount of radiant energy and thus cause a greater amount of gas formation by the puffing agent than do areas where this percentage is small, i.e., middle tone areas. Nonimage areas contain no pigment or at least only to an insignificant extent and so do not expand at least relative to the solid or middle tone areas.

The resulting sheet after light exposure, development, and high-intensity radiation exposure has a relief thickness corresponding to the tone of the photopolymer printing plate, i.e., thickest in solid tone areas (and of greatest thickness in the center of such areas), thinnest in nonprinting areas, and of essentially graduated thickness between these extremes.

To illustrate but not limit the invention, a number of drawings are set forth wherein:

FIG. 1 is a diagrammatic section through a makeready sheet of this invention.

FIG. 2 is a diagrammatic section of the makeready sheet of this invention after image exposure.

FIG. 3 is a diagrammatic section of the makeready sheet of this invention after image development.

FIG. 4 is a diagrammatic section of a source of high-intensity radiant energy and a makeready sheet selectively expanded in part.

FIG. 5 is a diagrammatic section of a printing plate having a selectively expanded makeready sheet in registered interlay position therewith and an impression cylinder.

It should be noted that the drawings are illustrative only, and it is not intended that the various layers and components of the novel makeready sheet material be represented in their true dimensions or proportions.

According to the preferred embodiment of my invention, designated for brevity as interlay makeready, a sheet such as illustrated in FIG. 1 as 24 comprising a carrier web or backing 20, a thermoexpansive layer 21, a diazo resin sensitizer layer 22, and a pigmented resinous overlayer 23 is first exposed to the same photographic negative to be used to produce the printing plate utilizing standard photographic exposure techniques. This exposure to actinic radiation yields the sheet material of FIG. 2 wherein the light-struck areas 28, 29, 30 are insolubilized, the unexposed areas remaining developable in selected solutions.

Exposed image area 28 is designated as a solid area, indicating a high tonal density, e.g., about 100% pigment is contained per unit surface area. Image areas 29 and 30 are to be considered middle tone areas of somewhat less percentage pigment per unit surface area. Additionally, area 29 is illustrated to have a higher degree of tonal density than area 30. For example, area 29 could have 75% pigment per unit surface area while area 30 could contain 60% pigment per unit surface area.

Development of the exposed FIG. 2 yields sheet material of FIG. 3 wherein the pigmented resinous overlayer 23 has been retained on the sheet overlying the exposed, insolubilized image diazo layer. The unexposed areas of

the diazo resin layer, along with the pigmented solvent-softenable resin overlayer directly overlying the unexposed areas have been selectively removed, leaving these areas relatively nonabsorptive of radiant energy.

After development of the image, the makeready sheet is briefly exposed to uniform and intense radiant energy as is illustrated by FIG. 4. In this figure, sheet material 24 with image areas 28, 29 and 30 facing toward high intensity radiation source 25 in elliptical reflector 26 is moved toward the right as indicated by the arrow, through the narrow focused band 27 of radiant energy. In those areas to the right of 27, the sheet is illustrated as being selectively expanded according to the pigmented imaged pattern thereon. Solid tone image area 28 is greatly expanded, while middle tone areas 29 and 30, of proportionately less total density, are expanded only to a degree commensurate with their tone. Nonimage areas 32 are unexpanded. Unexpanded image areas 31 to the left of the focused band or line 27 have not yet been exposed to the intense radiant energy.

In this high-intensity radiation exposure step, the pigmented image areas on the makeready sheet absorb infrared or equivalent radiant energy and become heated, which in turn heats areas of the layer of thermosoftenable resinous material and puffing agent adjacent thereto by conduction. These areas soften, the puffing agent in the layer is activated in the soft areas under these conditions of heat, and the gas released by the puffing agent produces bubbles in the softened areas causing them to swell. Upon cooling, the expanded areas become hard and the generated gas remains entrapped in the expanded areas of the layer.

In FIG. 5, an expanded makeready sheet 24 is illustrated in registered position beneath printing plate 39. Both are mounted on a suitable plate roller support 40. Selectively expanded areas 28, 29 and 30 of sheet 24 contact with solid tone area 34 and middle tone areas 33 and 35, respectively of printing form 39. A paper sheet 38 is shown receiving the inked image of printing form 39 by action of an impression cylinder 36 with packing layers 37 against the printing form.

#### DETAILED DESCRIPTION OF THE INVENTION

The flexible backing or carrier web is ideally between about 2 and 5 mils thick and should be dimensionally stable, i.e., resistant to curling, warping, stretching, etc., when overlaid with the thermoexpansive, light-sensitive, and pigmented layers. Preferably, the surface of the backing material to be overlaid should be of sufficient fibrous nature to assure that the thermoexpansive layer will be adequately anchored thereto. However, if a smooth surfaced backing is utilized, it may be roughened to secure the bonding thereto or a layer of adhesive may be deposited on the surface to effect bonding.

Preferred backing members are those characterized by low thermal conductivity, particularly when compared to the conductivity of metals, so that lateral diffusion of heat through the backing from adjacent portions of the bonded thermoexpansive layer during processing is minimized. Preferred backings are also light in color, since dark backings may be absorptive of the high intensity radiant energy encountered during processing.

In addition to the bleached kraft paper utilized in the illustrative example, generally those backings disclosed in the Gergen and Wartman patent are suitable. These include the nonfibrous films of glycol-terephthalate polymer, commercially known as "Mylar," cellulose acetate, silk screens, various laminates of materials, impregnated materials, etc.

The resinous materials and puffing agents disclosed by Gergen and Wartman to be useful in the thermoexpansive layer of their makeready sheet material are generally also useful in my invention.

The resinous material must be thermosoftenable but should possess sufficient toughness, hardness, and resilient

strength after processing of the makeready sheet to adequately resist compression from pressures encountered during letterpress printing operation.

These pressures are believed to approximate 250 p.s.i. for a period of about 15 seconds and a fully processed makeready sheet should be capable of maintaining at least a two mil difference in thickness between fully expanded and unexpanded areas under these operating conditions. Preferably, the thermoexpansive layer has a uniform, smooth, fused appearance prior to expansion.

Suitable resinous materials are usually polymeric, and preferably at least one hard thermoplastic polymeric material, i.e., having a Shore D Durometer hardness above about 40, is employed in the layer. However, softer materials which are temporarily thermoplastic but thermosetting or curable to suitable hardness in processing are also suitable either separately or in combination with a hard thermoplastic polymeric material.

The dispersed heat-sensitive puffing agent in the thermoexpansive layer should remain dispersed and stable at normal room temperature, i.e., 25° C. The puffing agent may react with or cure the thermosoftenable resinous material during processing or may even be a molecular component of the resinous material as long as the required ability to expand the layer under processing conditions hereinafter described is retained.

Preferred puffing agents chemically decompose at elevated temperature to yield a gas. However, puffing agents which vaporize upon heating, while inferior, can be suitable to use.

Finely pulverized, uniformly dispersed particles of a puffing agent facilitate the formation of a large number of tiny bubbles or cavities in the resinous layer with a great number of connecting columns of resin, all of which contributes to the strength and resiliency of expanded areas, as well as to the formation of well-regulated graduated relief patterns.

The amount of puffing agent employed may vary depending upon the relative ability of the agent to expand the sheet under the conditions employed in processing. A resinous layer may contain as little as approximately 1% by weight of a highly efficient puffing agent, e.g., "Celogen AZ," but may require up to approximately 30% by weight of a less efficient agent. Amounts in excess of approximately 10% by weight are generally to be avoided inasmuch as certain weaknesses are apt to develop within the sheet. However, an inefficient puffing agent which contributes to the strength of the sheet may be suitable to employ in high concentrations.

The temperature at which the resinous material softens and the temperature at which a puffing agent incorporated therein is activated should generally be within approximately the range of 75° F. of each other, although for some less critical combinations a temperature difference as great as about 150° F., or even greater, has been found useful. Generally, however, it has been found that if a puffing agent is activated at a temperature too far below that at which a resinous layer softens, control of expansion becomes difficult and desired graduated relief patterns are not easily obtained. If, on the other hand, the puffing agent is activated only at temperatures greatly above those at which the resinous material softens, difficulty arises with respect to retaining the released gas or other activating agent within the softened resinous layer. The faults of extremes are easily avoided if materials are selected with a view toward maintaining the activation temperature for the puffing agent reasonably close to the softening temperature of the resinous layer.

While solution or dispersion coating methods are adequate for application of the thermoexpansive layer to the backing, any method which will provide an essentially uniform film over the entire backing member is suitable, e.g., calendering, extruding, etc. The dry thickness of this layer is preferably between approximately two and seven mils, but may be as great as twelve mils or even greater with

satisfactory results. Layers greater than approximately twelve mils in thickness are generally undesirable because expanded areas may be compressible and expanded thickness differentials may be reduced. However, these disadvantages of a thick film may be corrected to some extent by incorporating suitable curing agents and/or thermosetting resins. A thickness of at least two mils is needed for the formation of proper relief patterns. Thinner coats fail to expand reliably and may even lose gas generated therein.

The applied thermoexpansive layer should preferably be dried to less than about 3% volatile solvent by weight so as to avoid unnecessary weaknesses in the layer upon expansion. Some minor amount of solvent can be advantageous, however, as serving to plasticize the resinous material to impart some planar stability to the sheet material, i.e., reduction of tendency to curl and warp.

When thermoplastic resins are utilized in the thermoexpansive layer, small amounts of organic, usually polymeric, plasticizers can also be advantageous to obtain planar stability. Such plasticizers, however, almost invariably reduce the strength of the expanded resinous layer. Accordingly, the thermoexpansive layer in such embodiments is generally at least about 3 mils thick, and preferably between 4 and 7 mils thick. This range affords the best results in terms of maintaining proper expanded thickness differentials under the conditions of printing press operation.

The light-sensitive sensitizer layer is composed of a light-sensitive diazo resin, which as a class is well known in the art. These resins insolubilize in areas exposed to actinic radiation relative to their initial unexposed areas. In general, any light-sensitive diazo resin which insolubilizes in light-exposed areas is useful in my invention.

Corona priming or treating of the sheet material prior to application of the diazo resin layer advantageously promotes wettability of the diazo application solution and adhesion of the insolubilized diazo to the thermoexpansive underlayer after imagewise exposure. Treatments of this nature are generally conventional procedures prior to overcoating of plastic surfaces.

Solution coating is a desirable method for application of the diazo resin sensitizer layer uniformly over the thermoexpansive layer of the makeready sheet material.

Because the diazo layer is extremely thin, applied coating weights generally being less than about 5 mg. per square foot, standard weight determination methods are generally unreliable and difficult to reproduce. For this reason, applied weights of the diazo resin can be most effectively measured optically, utilizing a Welsch Densitron with Kodak Wratten B-47 gelatin filter. When determined in this manner, utilizing the uncoated backing support as the reference or zero point, the applied coating weight expressed as reflected optical density should preferably be between about 0.25 and 0.60.

Optical densities of less than about 0.25 may not provide a uniform diazo sensitizer layer. As a result the pigmented, water-insoluble, solvent-softenable resinous overlayer may not adequately contact and bond to the diazo layer in light-exposed image areas or may not be adequately removed from the sheet material during image development. Optical densities greater than about 0.60, while not detrimental to image development, would be quite unnecessarily long image exposure times.

Application solution concentration, in terms of percent solids, of three to five percent has been found to be a generally usable range. Since the finished coating weight of this diazo layer is extremely light, use of a high solids concentration requires extremely close, perhaps unattainable, tolerances in application equipment. Judicious selection of solution concentration can be readily made by one skilled in the art depending upon the particular application equipment utilized.

Application solution solvents must be chosen so as not to exert a strong solvent action on the underlying

thermoexpansive layer. In general, lower aliphatic alcohols containing up to about four carbon atoms and aliphatic hydrocarbons containing up to about seven carbon atoms are suitable solvents in terms of their action on the underlying thermoexpansive layer, whereas aromatic hydrocarbons, esters, ketones, and chlorinated hydrocarbons are not suitable. Since a broad range of thermosoftenable resins are useful in that layer, a minor amount of experimentation may be necessary to determine suitability of particular solvents. One must begin with suitable solvents for the chosen diazo resin and determine which of these will not aggressively attack the thermoexpansive underlayer.

Applied over and in contact with the diazo sensitizer is a pigmented actinic light-transmittable continuous film or layer of a water-insoluble, solvent, softenable organic resin. In addition to providing a medium for pigment dispersion, this solvent-softenable organic resin should be one which bonds to the underlying diazo sensitizer in image-exposed areas, yet away clearly and sharply at the line of demarcation between image and non-image areas and is readily removed from the latter during development. While not knowing exactly why this phenomenon occurs, there is apparently a physical and/or chemical in situ bond formed between the diazo layer and pigmented resin overlayer on image exposure. Upon application of a developing solution which softens and permeates the resin overlayer, the solvent action on the unexposed diazo underlayer allows removal of the resin overlayer in unexposed areas.

Suitable organic resin compositions include various vinyl polymers, such as polyvinylbutyral, polymethylmethacrylate, polystyrene, polyvinyl acetate, polyethylene, polyvinylformal; condensation polymers such as polyester resins, e.g., alkyd resins, polyamide resins, phenolaldehyde resin, urealdehyde resins; other polymers such as cellulose acetate butyrate, polyalkylene-polysulfide resins, etc. In addition, compatible mixtures of the above-mentioned and other similar and equivalent resins can be used.

The pigment utilized in the organic resin/layer must provide high-intensity radiation absorptive image areas, and for this reason black or dark pigments, e.g., carbon black, are preferred. Pigment particle sizes of about five microns are preferred, thus some treatment of the pigment-resin dispersion, e.g., sand or ball milling, is generally required. Particle sizes greater than about ten microns may cause streaking or particle build-up during application of this layer, leading to non-uniformity.

Generally, the pigment concentration should be in the range of 80:20 to 55:45 parts by weight of resin to pigment, with 70:30 to 65:35 being preferred. Higher pigment concentrations tend to provide a structurally weak or brittle film or layer, i.e., it can be scratched, marred or cracked. Additionally, higher concentrations increase the opacity of the layer such that transmission of actinic light during image exposure becomes more difficult and undesirably long exposure time may be necessary. Too low a pigment concentration requires an increasingly thicker layer to provide adequate radiation absorption during expansion of the developed image.

A desirable method for uniformly applying the pigment dispersion to the diazo sensitizer layer is by conventional coating techniques. Since adequate absorptivity of high-intensity radiation is a requisite criteria for this pigmented layer, coating weights are generally couched more desirably in terms of optical density. Utilizing a Welsch Densichron with a Kodak wratten R-25 Gelatin filter and the uncoated backing support as a reference or zero point, optical densities should generally be in the preferred range of 0.90 to 1.30. Optical densities of less than 0.90 will generally not provide the selective absorption differential required to expand the makeready sheet uniformly and to the desired thickness after image development. Optical densities of greater than 1.30 make exposure of the diazo resin underlayer more difficult and time

consuming because of inadequate penetration of actinic light during image exposure. As a comparison, standard printer's ink has a comparable optical density in the range of 1.10 to 1.20.

5 A suitable solvent for the application of the pigmented resin layer is one which will adequately solvate the organic resin but not appreciably attack the diazo sensitizer layer and some minor experimentation may be necessary for optimum solvent selection. A range of two to five percent has been found adequate for solids concentration of the application solution. Too low a solids concentration may allow undesirable setting of the pigment dispersion and provide a nonuniform layer. An upper concentration limit is dependent on the application equipment available because increasingly thinner layers would be required.

10 The applied solvent-softenable pigmented resinous overlayer should preferably be dried to about 3% residual solvent. Image adhesion to the exposed diazo resin underlayer may be inadequate if the pigmented layer is too high in residual solvent. Generally, drying of the sheet material for up to about five minutes at about 180 to 200° F. will provide a sufficient degree of dryness in the pigmented layer.

15 In the processing of the novel makeready sheet material, conventional photographic techniques are acceptable for light exposure of the sheet material to the photographic negative.

20 Upon image exposure, the image must be properly developed. Solutions used to imagewise develop the light-exposed makeready sheet material should have certain characteristics. Preferably, the solution should exert a slight but not vigorous solvent or swelling action on the pigmented overlayer composition. Additionally, it should be an active solvent for the unexposed diazo sensitizer but have little or no effect on the light-reacted sensitizer or the thermoexpansive underlayer. Ordinarily, a mixture of two or more preferably miscible liquids is necessary to provide a developing solution having these desirable characteristics. An operable developing solution can be found for any combination of thermoexpansive layer, diazo sensitizer layer, and pigmented resinous layer employed, although some amount of experimentation may be required. Generally, a suitable developing solution can be obtained by combining a solvent which exerts at least a partial solvent or swelling action on the pigmented resinous overlayer with a second solvent, miscible with the first, which is not a solvent for the pigmented resinous overlayer, one of the two being a solvent for the unexposed diazo composition. Neither of the two solvents, nor the mixtures thereof should be a solvent for the exposed diazo composition. If the first solvent aggressively attacks the pigmented resinous overlayer, it should be diluted with a second component, such that the solvent action of the mixture is not vigorous.

25 30 35 40 45 50 55 Conventional diazo resin sensitizers are generally at least somewhat water-soluble prior to light exposure. Since both the thermoexpansive layer and the pigmented resinous overlayer are generally water-insoluble, water may be a suitable component for a developing solution.

60 Other components and processing solutions may be arrived at by judicious selection, such as the 1:1 by volume normal propanol-water developing solution of the illustrative example. Neither water nor normal propanol by themselves exert any substantial solvent action on the polyvinyl formal resin overlayer.

65 After image development, the makeready sheet material is comparable to the inked makeready sheet material of the Gergen and Wartman patent. Consequently, the equipment and conditions for image expansion utilized in Gergen and Wartman are equally applicable for the makeready sheet material of my invention.

70 75 The preferred temperature range of which expansion of the heat-sensitive thermoexpansive layer occurs is well above room temperature and is between approximately 150 and 350° F., but may be as high as 450° F. or even

considerably higher. Expansion at exceedingly low temperatures is generally unreliable and uncontrollable. Conversely, expansion at temperatures above about 450° F. or 500° F. creates problems with respect to suitable exposure conditions for processing as well as with respect to obtaining suitable graduated relief patterns.

Having described my invention in a general manner, the same is illustrated by the following nonlimiting example, wherein all parts are by weight unless otherwise specified.

#### EXAMPLE

A solution is first prepared for the thermoexpansible layer by mixing the following:

| Parts                                                                                                                              |       |
|------------------------------------------------------------------------------------------------------------------------------------|-------|
| VXDV, a tradename for a dispersion grade vinyl chloride-vinyl acetate copolymer, available from the Union Carbide Co.              | ----- |
| 50                                                                                                                                 |       |
| Pliovic A0-2, a trade name for a vinyl terpolymer available from the Goodyear Chemical Co.                                         | ----- |
| 50                                                                                                                                 |       |
| EPON 828, a trade name for an epoxy condensation polymer of epichlorohydrin and bisphenol A, available from the Shell Chemical Co. | ----- |
| 20                                                                                                                                 |       |
| Diphthalyl dihydrazide, a curing agent for the epoxy resin                                                                         | ----- |
| 30                                                                                                                                 |       |
| Celogen AZ, a trade name for azodicarbonamide, available from the U.S. Rubber Co.                                                  | ----- |
| 25                                                                                                                                 |       |
| Primary amyl acetate                                                                                                               | ----- |
| 5                                                                                                                                  |       |
| Naphtha                                                                                                                            | ----- |
| 53.5                                                                                                                               |       |
|                                                                                                                                    | 28.1  |

The VXDV and the Pliovic A0-2 have fusion temperatures of about 300° F. The diphthalyl dihydrazide is a highly effective curing agent for epoxy resins at the temperature utilized during expansion. The Celogen AZ puffing agent releases nitrogen gas on decomposition, starting at about 285° F.

This mixture is coated onto a 44 pound bleached Kraft machine calendered paper at a 12 mil orifice setting and dried for 3 minutes at room temperature followed by 3 minutes at 180° F.

The layer is then fused for 5 minutes at about 265° F., leaving a residual solvent of 2-3 percent by weight in the layer.

This coated sheet material is then corona treated at a web speed of 50 feet per minute, utilizing a 70 volt, 9-10 ampere input with a  $\frac{3}{16}$  inch gap.

A solution of a light-sensitive diazo resin sensitizer is prepared under subdued light by dissolving:

| Parts                                                                                              |       |
|----------------------------------------------------------------------------------------------------|-------|
| Aromatic sulfonic acid salt of the condensation product of 4-diazo diphenylamine acid formaldehyde | ----- |
| 4                                                                                                  | 50    |
| Methyl Cellosolve                                                                                  | ----- |
| 96                                                                                                 |       |

This solution is coated over the thermoexpansible layer at a 3 mil orifice setting and dried for 7 minutes at 180° F.

The optical density of the coating is measured with a Welsch Densichron equipped with a Kodak wratten B-47 Gelatin filter utilizing uncoated backing as the reference point. This density is 0.42.

A solution of a water-insoluble, solvent-softenable resin is prepared by mixing:

| Parts                                                                                            |       |
|--------------------------------------------------------------------------------------------------|-------|
| Formvar 15/95E, a tradename for a polyvinylformal resin available from the Monsanto Chemical Co. | ----- |
| 7                                                                                                |       |
| Methyl butynol                                                                                   | ----- |
| 90                                                                                               |       |

To this solution is added 3 parts Regal 300, a carbon black available from the Cabot Co.

This dispersion, containing a 70:30 weight ratio of resin to pigment, is passed through a sand mill until maximum particles size is about 10 microns, coated over the diazo sensitizer layer at a 3 mil orifice setting, and dried for 4 minutes at 190° F.

The optical density of the resultant sheet, measured with a Welsch Densichron equipped with a Kodak wratten R-25 Gelatin filter, is 1.0 utilizing uncoated backing as the reference point.

The makeready sheet material is then exposed through a photographic negative of the desired printed matter to a carbon arc (Grafarc Type 33500-24) for 2 minutes at a distance of 36 inches.

5 The light-exposed sheet is placed on a smooth surface and a small amount of a 1:1 by volume solution of normal propanol and water is spread over the entire sheet. The sheet is wiped in a circular motion with soft cotton or a conventional lithographic plate developing pad, whereupon the unexposed diazo layer and corresponding pigmented overlayer are removed. The sheet is then wiped dry.

10 This image-developed sheet is exposed to high-intensity radiation in a commercially available Model MR-2 Make-ready Machine, available from the Minnesota Mining and Manufacturing Company. This machine has a 3000 watt radiant energy source at a power input of 480 volts. At a focused band width of approximately  $\frac{3}{16}$  inch, the sheet material is passed once through the machine at a speed of 7.0 (corresponding to about 32 inches per minute).

15 In solid tone image areas the sheet material is expanded to a total thickness of 11.5 mils, 4.5 mils above unexpanded areas. Other areas are expanded commensurate with their tone. For example, in an area of 50 percent printing elements (50 percent being nonprinting) expansion is to about 9.5 mils, 2.5 mils above the unexpanded areas. The fully processed sheet thus presents a thickness relief corresponding to the tone of the printing plate.

20 The following table will further illustrate appropriate developing solutions for sheet constructions containing the thermoexpansible layer and diazo layer of the preceding example. In all cases the pigment utilized is that of the example and the dispersion application solvent is methyl butynol. Where indicated in the developing solutions, ratios are by volume.

25 Overcoating resin composition: Developing solution  
Butvar B-98, trade name for polyvinyl butyral, available from the Monsanto Chemical Co. ----- Ethanol-water 7:3 ratio.

30 Gelva V-60, trade name for polyvinyl acetate, available from the Monsanto Chemical Co. ----- n-Propanol-water 1:3 ratio.

35 Elvacite 20-42, trade name for an acrylate resin available from E. I. du Pont de Nemours Company ----- Isopropanol-water 6:4 ratio.

40 What is claimed is:

45 1. A presensitized, light-sensitive, flexible sheet material of essentially uniform thickness adaptable for makeready in letterpress printing, said sheet material comprising:

50 (a) a flexible carrier web;  
(b) a selectively thermoexpansible layer at least 2 mils thick overlying said carrier web, comprising an at least temporarily thermosoftenable resinous material, and uniformly distributed therethrough a normally dormant, heat-sensitive puffing agent activatable at a temperature well above room temperature to expand said layer under conditions of heat, said puffing agent being present in an amount sufficient to provide on rapid and complete heat activation of said layer an increase of at least 2 mils in the thickness thereof;

55 (c) a light-sensitive diazo resin sensitizer layer overlying said thermoexpansible layer and in direct contact therewith, said sensitizer layer upon exposure to actinic light becoming selectively insolubilized and firmly bonded to said thermoexpansible underlayer in exposed areas;

60 (d) a thin, continuous layer overlying said diazo resin underlayer and in direct contact therewith comprising

## 11

a water-insoluble, solvent-softenable resinous polymer, and uniformly distributed therethrough a finely divided pigment, said layer being actinic light-transmittable and selectively removable together with underlying diazo resin layer in areas where said diazo resin layer is unexposed to actinic light, said layer being firmly bonded to said underlying diazo resin layer in light-exposed areas and absorptive of high intensity radiant energy; said sheet material in expanded condition being capable of supporting pressures of at least on the order of 250 p.s.i. for about 15 seconds while maintaining areas of maximum expansion at least approximately 2 mils greater than the initial thickness thereof.

2. The article of claim 1 in which the selectively thermoexpansive layer contains a thermosetting resin.

3. The article of claim 2 in which the selectively thermoexpansive layer contains a curing agent for said thermosetting resin.

4. The article of claim 2 in which the selectively thermoexpansive layer is at least about 3 mils thick and contains an organic plasticizer.

5. A presensitized, light-sensitive, flexible sheet material of essentially uniform thickness adaptable for make-ready in letterpress printing, said sheet material comprising:

(a) a flexible carrier web;  
 (b) a selectively thermoexpansive layer at least 2 mils thick overlying said carrier web, comprising a thermoplastic resin, a thermosetting resin, and a curing agent for said thermosetting resin, and uniformly distributed therethrough a normally dormant, heat-sensitive puffing agent activatable at a temperature well above room temperature to expand said layer under conditions of heat, said puffing agent being present in an amount sufficient to provide on rapid and complete heat activation of said layer an increase of at least 2 mils in the thickness thereof;

(c) a light-sensitive diazo resin sensitizer layer overlying said thermoexpansive layer and in direct contact therewith, said sensitizer layer upon exposure to actinic light becoming selectively insolubilized and firmly bonded to said thermoexpansive underlayer in exposed areas;

(d) a thin, continuous layer overlying said diazo resin underlayer and in direct contact therewith comprising a water-insoluble, solvent-softenable resinous polymer, and uniformly distributed therethrough a finely divided pigment, said layer being actinic light-transmittable and selectively removable together with underlying diazo resin layer in areas where said diazo resin layer is unexposed to actinic light, said layer being firmly bonded to said underlying diazo resin layer in light-exposed areas and absorptive of high intensity radiant energy;

said sheet material in expanded condition being capable of supporting pressures of at least on the order of 250 p.s.i. for about 15 seconds while maintaining areas of maximum expansion at least approximately 2 mils greater than the initial thickness thereof.

6. The article of claim 5 wherein said water-insoluble, solvent-softenable resinous polymer is polyvinyl-formal.

## 12

7. The article of claim 5 wherein said finely divided pigment is carbon black.

8. A process of preparing a makeready sheet suitable for letterpress printing comprising:

5 (1) exposing to actinic light through a photographic negative or transparency a light-sensitive flexible sheet material comprising:

(a) a flexible carrier web;

(b) a selectively thermoexpansive layer at least 2 mils thick overlying said carrier web, comprising an at least temporarily thermosoftenable resinous material, and uniformly distributed therethrough a normally dormant, heat-sensitive puffing agent activatable at a temperature well above room temperature to expand said layer under conditions of heat, said puffing agent being present in an amount sufficient to provide on rapid and complete heat activation of said layer an increase of at least 2 mils in the thickness thereof;

(c) a light-sensitive diazo resin sensitizer layer overlying said thermoexpansive layer and in direct contact therewith, said sensitizer layer upon exposure to actinic light becoming selectively insolubilized and firmly bonded to said thermoexpansive underlayer in exposed areas;

(d) a thin, continuous layer overlying said diazo resin underlayer and in direct contact therewith comprising a water-insoluble, solvent-softenable resinous polymer, and uniformly distributed therethrough a finely divided pigment, said layer being actinic light-transmittable and selectively removable together with underlying diazo resin layer in areas where said diazo resin layer is unexposed to actinic light, said layer being firmly bonded to said underlying diazo resin layer in light-exposed areas and absorptive of high intensity radiant energy;

(2) selectively developing said light-exposed sheet material in an imagewise manner to remove areas of (c) and (d) unexposed to said actinic light;

(3) exposing said developed sheet material to uniform high-intensity radiant energy, said radiant energy being differentially absorptive in image areas commensurate with the tonal density of said image areas, said radiant energy providing a heat pattern sufficient to selectively expand said sheet material in accordance with said heat pattern at least 2 mils greater than the initial thickness thereof.

## References Cited

## UNITED STATES PATENTS

|           |         |                 |       |           |
|-----------|---------|-----------------|-------|-----------|
| 2,825,282 | 4/1958  | Gergen et al.   | ----- | 101—401.3 |
| 3,298,833 | 1/1967  | Gaynor          | ----- | 96—75 X   |
| 3,391,637 | 7/1968  | Reynolds et al. | ----- | 101—401.3 |
| 3,410,686 | 11/1968 | Prater          | ----- | 96—75 X   |

DAVID KLEIN, Primary Examiner

60 U.S. CL. X.R.

96—75; 101—401.3